

## UNITED STATES PATENT OFFICE

2,130,507

## HIGH MOLECULAR WEIGHT ISO-OLEFINE POLYMERS AND PROCESS OF PRODUCING THE SAME

Michael Otto and Martin Mueller-Cunradi, Ludwigshafen-on-the-Rhine, Germany, assignors to I. G. Farbenindustrie Aktiengesellschaft, Frankfort-on-the-Main, Germany

No Drawing. Original application July 21, 1932, Serial No. 623,812. Divided and this application April 2, 1935, Serial No. 14,273. In Germany July 25, 1931

## 7 Claims. (Cl. 260—2)

The present invention relates to the preparation of valuable hydrocarbon products, more particularly those of higher boiling point.

We have found that hydrocarbon mixtures, in particular those having a boiling point above 200° C., and especially those boiling above about 325° C. at ordinary pressure, for example lubricating oils or greases or hard or soft paraffin wax, are considerably improved and that in particular the viscosity of these materials is much increased by adding thereto high molecular hydrocarbons having a molecular weight of for example 1000 or 2000 or even more, which are obtained by polymerizing iso-olefines and in particular iso-butylene.

By the addition of these high molecular hydrocarbons obtained by polymerizing iso-olefines (which hydrocarbons for the sake of brevity are hereinafter referred to as polymerized iso-olefines) also the temperature-viscosity curve of the hydrocarbon mixtures to be improved is remarkably flattened in many cases. Furthermore the electric properties of these hydrocarbon mixtures are considerably changed so that for example by the addition of only 1 per cent of polymerized iso-olefines the disruptive strength of the hydrocarbon mixtures is increased to double its height and that this effect even remains after artificial ageing. The hydrocarbon mixtures so improved may therefore be employed with great advantage as insulating oils for transformers and switches. Hard and soft paraffin wax is rendered transparent by the addition of the said polymerized iso-olefines; furthermore the formation of fissures and cracks is prevented thereby. In many cases it is sufficient to add the polymerized iso-olefines in an amount of from a fraction of none per cent up to about 10 per cent with reference to the hydrocarbon mixtures to be improved, but the amount added may also be much higher, as for example about 20 or 35 or even 50 per cent.

For many purposes, as for example for lubricating automobile motors, it is well known that oils are necessary which on the one hand still have a satisfactory viscosity at high temperatures, as for example from 100° to 150° C., and on the other hand are still so thinly liquid at low temperatures that the friction is not too great for the automobile motor to be set in motion directly by the starting device. According to the present invention oils can be prepared which correspond to a great extent to these requirements and which are far superior to the special automobile oils hitherto in commerce.

The effect of the addition of the said polymer-

ized iso-olefines is shown in the following table of examples. The oils used in experiments A, B, C, D and E are mineral oils of the type of the commercial light to medium machine oils. Experiments A', B', C', C'', D' and E' show the effect of the addition of an iso-butylene polymerization product. Experiments F, G and H are the tests of special automobile oils. In all cases the temperatures are given in degrees C.

The viscosity index indicates the value of the oil in that as the index value increases, the quality of the oil improves.

| Experiment | Percentage iso-butylene polymerization product | Viscosity in degrees Engler at— |      |      |      |      |           | 15 |
|------------|------------------------------------------------|---------------------------------|------|------|------|------|-----------|----|
|            |                                                | 0°                              | 20°  | 38°  | 50°  | 100° | 150°      |    |
| A          | 0                                              | 125                             | 25   | 8.3  | 8.8  | 1.6  | Below 1.2 |    |
| A'         | 6                                              | 170                             | 42   | 15.6 | 8.8  | 2.25 | 1.44      | 20 |
| B          | 0                                              | 46                              | 11   | 5.3  | 3.0  | 1.45 | Below 1.2 |    |
| B'         | 4                                              | 98                              | 29.5 | 12.9 | 7.7  | 2.25 | 1.47      |    |
| C          | 0                                              | —                               | —    | 3.3  | 2.1  | 1.3  | —         |    |
| C'         | 4                                              | 110                             | 33   | 13.9 | 8.2  | 2.32 | 1.48      |    |
| C''        | 13                                             | 280                             | 84   | 35.2 | 21.8 | 5.0  | 2.18      |    |
| D          | 0                                              | 12                              | 4.8  | 2.55 | 2.0  | 1.3  | —         |    |
| D'         | 6                                              | 55                              | 20.5 | 9.8  | 6.5  | 2.25 | 1.52      | 25 |
| E          | 0                                              | 225                             | 41   | 12.9 | 7.0  | 1.8  | 1.22      |    |
| E'         | 1                                              | About 58                        | 19.1 | 10.3 | 2.3  | 1.42 | —         |    |
| F          | 0                                              | 280                             | —    | —    | —    | —    | 1.4       |    |
| F          | 0                                              | About                           | 63   | 20.2 | 11.1 | 2.3  | —         |    |
| G          | 0                                              | 300                             | —    | —    | —    | —    | 1.32      |    |
| G          | 0                                              | Over                            | 73.5 | 21.8 | 11   | 2.12 | —         |    |
| H          | 0                                              | 300                             | 83   | 25.3 | 13   | 2.5  | 1.45      | 30 |
| H          | 0                                              | Over                            | —    | —    | —    | —    | —         |    |

| Experiment | Viscosity index | Setting point | Flash point | Density at 20° | 35 |
|------------|-----------------|---------------|-------------|----------------|----|
|            |                 |               |             |                |    |
| A          | 60              | 8             | 242         | 0.880          |    |
| A'         | 120             | 13            | 242         | 0.880          |    |
| B          | 40              | 6             | 215         | 0.870          |    |
| B'         | 134             | 12            | 215         | 0.870          |    |
| C          | —               | 50            | 180         | 0.885          | 41 |
| C'         | 134             | 45            | 180         | 0.885          |    |
| D          | —               | 9             | 185         | 0.860          |    |
| D'         | Over 140        | 12            | 185         | 0.860          |    |
| E          | 67              | 2.5           | 221         | 0.914          |    |
| E'         | 105             | 5             | 222         | 0.914          |    |
| F          | 104             | 7             | 234         | 0.883          |    |
| G          | 65              | 16            | 235         | 0.901          | 45 |
| H          | 98              | —             | —           | —              |    |

From the table it can be seen that the addition of the highly polymerized isobutylene products considerably improves the oils. The resulting improved oils have even a higher viscosity index than special automobile oils of high value.

On account of the low coke test of the polymerized iso-olefines the lubricating oils the vis-

cosity of which has been increased by the addition of the said polymerized iso-olefines instead of by the addition, hitherto usual, of hot steam cylinder oils or bright stock oils, have a very low coke test. This will be illustrated by the following table showing the viscosity and the Conradson coke test of a special winter oil without and with additions increasing the viscosity:

| 10 | Additions                                | Viscosity at 100° C. | Conradson coke test |
|----|------------------------------------------|----------------------|---------------------|
| 15 | 4.6 per cent of polymerized iso-butylene | 1.56                 | 0.08                |
|    | 33.0 per cent of bright stock oil        | 3.0                  | 0.09                |
| 15 | 33.0 per cent of hot steam cylinder oil  | 1.9                  | 0.52                |
|    |                                          | 1.9                  | 0.71                |

The effect of the addition of polymerized iso-olefines to greases is shown by the following example:

20 1200 grams of a lubricating oil for freezing machines having a viscosity of 7° Engler at 20° C. and a setting point of 45° below zero C. is mixed after dissolution therein of 60 grams of polymerized iso-butylene with 250 grams of oleic acid glyceride, 30 grams of hydrate of lime and 20 grams of a 20 per cent solution of caustic soda, the mixture being stirred for about 5 hours at 100° C. The resulting grease is soft and of a great adhesive power.

30 Also hard and soft paraffin wax is considerably improved by the addition of polymerized iso-butylene as will be seen from the following example:

35 Polymerized iso-butylene is added in an amount of from 1 to 4 per cent to paraffin wax having a strong tendency to form crystals and which when employed for casting candles causes the formation of fissures. The candles cast with the mixture thus obtained do not show fissures 40 to a substantial degree and fissures or points of crystallization still formed disappear after 1 or 2 days. The candles are uniformly transparent.

45 The production of the polymerized iso-olefines to be added to the hydrocarbon products is effected by polymerization of the iso-olefines in the presence of suitable catalysts, preferably volatilizable inorganic halides, such as boron fluoride, boron fluoride charged with hydrofluoric acid, phosphorus trifluoride, phosphorus pentafluoride, 50 aluminium chloride, preferably in statu nascendi, such as aluminium chloride as is formed by allowing hydrogen chloride to act on aluminium, or solutions or double compounds of the said halides, while cooling so strongly that no sudden 55 substantial increase in temperature occurs. The said catalysts may be employed as such or together with substances such as phenol or cresol, in which they dissolve without decomposition, whether with the formation of real solutions, or 60 with the formation of double compounds. The strong cooling prevents the undesired too rapid reaction, which leads to products not having the desired molecular weight, and furthermore the loss in iso-butylene which would occur by a sudden superheating. It may be advantageous not to bring the catalyst into contact with the iso-butylene at once but gradually. By moving the iso-butylene, for example by stirring, the removal of the reaction heat is favoured and local 65 superheating is avoided. The polymerization of iso-butylene is a strongly exothermic reaction.

70 Corresponding to the different intensity of the catalytic action of the different catalysts it is necessary to vary the intensity of cooling. For 75 example, in the employment of the extremely

active boron fluoride it is necessary to keep the temperature during the reaction below 5° C. Temperatures as low as 10° below zero C. or still lower temperatures may be employed.

The cooling may be effected externally by means of cooling baths or internally by adding to the reacting substances cold materials which have no favourable influence on the reaction, as for example solid carbon dioxide.

10 The catalysts may be employed in very small amounts; for example less than 1 per cent of catalyst is sufficient when boron fluoride is employed. It is, however, possible to use also higher percentages of catalysts, for example 3 or 5 per cent of aluminium chloride.

15 Solvents, such as pentane, may be present during the reaction. The resulting product is very viscous and of a from sticky to semi-solid or solid or rubber-like consistency; it is colorless and clear, soluble in liquid hydrocarbons in any proportion and may easily be depolymerized, without the formation of coke, to form gaseous and lower boiling hydrocarbons by heating, for example to a temperature of 300° C. Of particular value are the polymerized products having a 20 molecular weight of more than 2,000, as for example up to 10,000 and more. The Conradson-coke-test of these products is very low and not far from zero; it amounts for example to 0.01.

25 The following examples further illustrate the preferred preparation of the said polymerized iso-olefines; the preparation of these products is, however, not restricted to the particular operations there described.

#### Example 1

35

About 0.5 part of boron fluoride is led into 100 parts of liquid iso-butylene which is cooled by a bath of carbon dioxide at 80° below zero C. The polymerization soon sets in vigorously. By intense stirring while maintaining the cooling, the considerable heat of reaction is led away so well that the temperature does not rise above 20° below zero C. The reaction product has a mean 40 molecular weight of 3500. It is extremely viscous, may be drawn out into long threads and, even at 200° C., it is still not liquid.

#### Example 2

45

The process is similar to that in Example 1 except that before and during the leading in of boron fluoride solid carbon dioxide is thrown into the reaction material in order to maintain the temperature below from 60° to 70° below zero C. A product having a mean molecular weight of 50 about 5000 is obtained. The product is as viscous as normal rubber masticated at 70° C. It is slightly sticky, colorless and clear.

#### Example 3

55

A 20 per cent solution of iso-butylene in pentane is kept at 40° below zero C. while leading in boron fluoride. After expelling volatile constituents with steam the product has a molecular weight of 2500. The product is much more soft and more sticky than that obtained according to Example 2; it is colorless and clear and may be drawn into long threads.

#### Example 4

60

A mixture of 110 grams of iso-butylene and 110 grams of normal butylene (mainly  $\alpha$ -butylene) is polymerized as described in Example 2. After 65 distilling off the normal butylene 120 grams of a 70

75

residue having a molecular weight of about 4000 are obtained.

*Example 5*

5 A mixture of 50 grams of iso-butylene and 250 grams of normal butylene are polymerized as described in Example 2. After distilling off a residue of 58 grams is obtained. From this residue 11 grams may be distilled off under a pressure of 0.1 millimeter mercury gauge and at a 10 temperature up to 200° C., 47 grams of a product having a molecular weight of about 3000 thus being obtained.

*Example 6*

15 A mixture consisting of 900 grams of natural gas gasoline (distilling almost completely up to 60° C.), 60 grams of iso-butylene and 290 grams of normal butylene, which mixture is liquid under a slight superatmospheric pressure, is polymerized as described in Example 2.

20 After distilling off 79 grams of a polymerization product are obtained, of which 16 grams, under a pressure of 15 millimeters mercury gauge, boil up to 200° C., and further 18 grams boil up to this temperature, under a pressure of 0.07 millimeter mercury gauge, 45 grams of a residue having a mean molecular weight of 3500 remain in the still.

25 The molecular weight may be increased by depolymerizing either the said 79 grams of polymerization product or the said grams of residue into iso-butylene by heating, if desired, in the presence of catalysts and then again polymerizing the depolymerized products. For example the 30 said polymerization product or the said residue is heated to a temperature of 300° C. in the presence of phosphoric acid while allowing the condensable vapors evolved from the heating zone to return. The resulting iso-butylene, when polymerized as described in Example 2 furnishes a 35 polymerization product having a molecular weight of more than 5000.

40 This application has been divided out from our 45 copending application Ser. No. 623,812 filed July 21st, 1932.

What we claim is:—

1. The process of producing a high molecular 50 polymerization product of an iso-olefine which comprises polymerizing an iso-olefine in the presence of a volatilizable inorganic halide polymerization catalyst while continuously maintaining the temperature of the reaction mixture below 10° below zero C. throughout the reaction 55 period.

CERTIFICATE OF CORRECTION

Patent No. 2,130,507.

September 20, 1938.

MICHAEL OTTO, ET AL.

It is hereby certified that error appears in the printed specification of the above numbered patent requiring correction as follows: Page 3, second column, line 30, claim 5, for the claim reference numeral "3" read 1; line 39, claim 6, for the claim reference numeral "4" read 2; and that the said Letters Patent should be read with this correction therein that the same may conform to the record of the case in the Patent Office.

Signed and sealed this 6th day of December, A. D. 1938.

Henry Van Arsdale

2. The process of producing a high molecular polymerization product of iso-butylene which comprises polymerizing iso-butylene in the presence of a volatilizable inorganic halide polymerization catalyst while continuously maintaining the temperature of the reaction mixture below 10° below zero C. throughout the reaction period. 5

3. The process of producing a high molecular polymerization product of an iso-olefine which comprises polymerizing an iso-olefine in the presence of boron fluoride while continuously maintaining the temperature of the reaction mixture below 10° below zero C. throughout the reaction period. 10

4. The process of producing a high-molecular 15 polymerization product of iso-butylene which comprises polymerizing iso-butylene in the presence of boron fluoride while continuously maintaining the temperature of the reaction mixture below 10° below zero C. throughout the reaction period. 20

5. A polymerization product of an aliphatic 25 iso-olefine which is, substantially saturated, and has a from viscous, sticky to solid consistency at ordinary temperature, which product by heating is depolymerizable to gaseous or low boiling hydrocarbons without substantial formation of coke, which has a molecular weight of more than 3000 and which is soluble in liquid hydrocarbons in any proportion obtained according to the process 30 of claim 3.

6. A polymerization product of iso-butylene 35 which is substantially saturated, and has a from viscous, sticky to solid consistency at ordinary temperature, which product by heating is depolymerizable to gaseous or low boiling hydrocarbons without substantial formation of coke, which has a molecular weight of more than 3000 and which is soluble in liquid hydrocarbons in any proportion obtained according to the process of claim 4. 40

7. The process of producing a high molecular 45 polymerization product of an iso-olefine which comprises polymerizing an iso-olefine in the presence of a volatilizable inorganic halide polymerization catalyst selected from the class consisting of boron fluoride, boron fluoride charged with hydrofluoric acid, phosphorous trifluoride, phosphorous pentafluoride, aluminum chloride and the double compounds of said halides, while continuously maintaining the temperature of the reaction mixture below 10° below zero C. throughout the reaction period. 50

MICHAEL OTTO.  
MARTIN MUELLER-CUNRADI. 55

residue having a molecular weight of about 4000 are obtained.

*Example 5*

5 A mixture of 50 grams of iso-butylene and 250 grams of normal butylene are polymerized as described in Example 2. After distilling off a residue of 58 grams is obtained. From this residue 11 grams may be distilled off under a pressure of 0.1 millimeter mercury gauge and at a 10 temperature up to 200° C., 47 grams of a product having a molecular weight of about 3000 thus being obtained.

*Example 6*

15 A mixture consisting of 900 grams of natural gas gasoline (distilling almost completely up to 60° C.), 60 grams of iso-butylene and 290 grams of normal butylene, which mixture is liquid under a slight superatmospheric pressure, is polymerized as described in Example 2.

20 After distilling off 79 grams of a polymerization product are obtained, of which 16 grams, under a pressure of 15 millimeters mercury gauge, boil up to 200° C., and further 18 grams boil up to this temperature, under a pressure of 0.07 millimeter mercury gauge, 45 grams of a residue having a mean molecular weight of 3500 remain in the still.

25 The molecular weight may be increased by depolymerizing either the said 79 grams of polymerization product or the said grams of residue into iso-butylene by heating, if desired, in the presence of catalysts and then again polymerizing the depolymerized products. For example the 30 said polymerization product or the said residue is heated to a temperature of 300° C. in the presence of phosphoric acid while allowing the condensable vapors evolved from the heating zone to return. The resulting iso-butylene, when polymerized as described in Example 2 furnishes a 35 polymerization product having a molecular weight of more than 5000.

40 This application has been divided out from our 45 copending application Ser. No. 623,812 filed July 21st, 1932.

What we claim is:—

1. The process of producing a high molecular 50 polymerization product of an iso-olefine which comprises polymerizing an iso-olefine in the presence of a volatilizable inorganic halide polymerization catalyst while continuously maintaining the temperature of the reaction mixture below 10° below zero C. throughout the reaction 55 period.

CERTIFICATE OF CORRECTION

Patent No. 2,130,507.

September 20, 1938.

MICHAEL OTTO, ET AL.

It is hereby certified that error appears in the printed specification of the above numbered patent requiring correction as follows: Page 3, second column, line 30, claim 5, for the claim reference numeral "3" read 1; line 39, claim 6, for the claim reference numeral "4" read 2; and that the said Letters Patent should be read with this correction therein that the same may conform to the record of the case in the Patent Office.

Signed and sealed this 6th day of December, A. D. 1938.

Henry Van Arsdale

2. The process of producing a high molecular polymerization product of iso-butylene which comprises polymerizing iso-butylene in the presence of a volatilizable inorganic halide polymerization catalyst while continuously maintaining the temperature of the reaction mixture below 10° below zero C. throughout the reaction period. 5

3. The process of producing a high molecular polymerization product of an iso-olefine which comprises polymerizing an iso-olefine in the presence of boron fluoride while continuously maintaining the temperature of the reaction mixture below 10° below zero C. throughout the reaction period. 10

4. The process of producing a high-molecular 15 polymerization product of iso-butylene which comprises polymerizing iso-butylene in the presence of boron fluoride while continuously maintaining the temperature of the reaction mixture below 10° below zero C. throughout the reaction period. 20

5. A polymerization product of an aliphatic 25 iso-olefine which is, substantially saturated, and has a from viscous, sticky to solid consistency at ordinary temperature, which product by heating is depolymerizable to gaseous or low boiling hydrocarbons without substantial formation of coke, which has a molecular weight of more than 3000 and which is soluble in liquid hydrocarbons in any proportion obtained according to the process 30 of claim 3.

6. A polymerization product of iso-butylene 35 which is substantially saturated, and has a from viscous, sticky to solid consistency at ordinary temperature, which product by heating is depolymerizable to gaseous or low boiling hydrocarbons without substantial formation of coke, which has a molecular weight of more than 3000 and which is soluble in liquid hydrocarbons in any proportion obtained according to the process of claim 4. 40

7. The process of producing a high molecular 45 polymerization product of an iso-olefine which comprises polymerizing an iso-olefine in the presence of a volatilizable inorganic halide polymerization catalyst selected from the class consisting of boron fluoride, boron fluoride charged with hydrofluoric acid, phosphorous trifluoride, phosphorous pentafluoride, aluminum chloride and the double compounds of said halides, while continuously maintaining the temperature of the reaction mixture below 10° below zero C. throughout the reaction period. 50

MICHAEL OTTO.  
MARTIN MUELLER-CUNRADI. 55

## CERTIFICATE OF CORRECTION.

Patent No. 2,130,507.

September 20, 1938.

MICHAEL OTTO, ET AL.

It is hereby certified that error appears in the printed specification of the above numbered patent requiring correction as follows: Page 2, first column, line 63, before the word "molecular" insert high; and second column, line 8, for "favourable" read unfavourable; and that the said Letters Patent should be read with this correction therein that the same may conform to the record of the case in the Patent Office.

Signed and sealed this 16th day of May, A. D. 1939.

(Seal)

Henry Van Arsdale  
Acting Commissioner of Patents.